

June 5, 1934.

C. G. MAIER

1,961,424

ZINC REFINING PROCESS

Filed Dec. 26, 1931

2 Sheets-Sheet 1



Inventor

Charles G. Maier,

By Mueller & McLaughlin Atq. 1

June 5, 1934.

C. G. MAIER

1,961,424

ZINC REFINING PROCESS

Filed Dec. 26, 1931

2 Sheets-Sheet 2



## UNITED STATES PATENT OFFICE

1,961,424

## ZINC REFINING PROCESS

Charles G. Maier, Berkeley, Calif.

Application December 26, 1931, Serial No. 583,246

3 Claims. (Cl. 75—28)

My invention relates in general to the reduction of zinc ores. It relates more in particular to improved means and the process for reducing zinc oxide to metallic zinc, and is a continuation in part of my prior application, Serial Number 513,458, filed February 4, 1931.

In the known art, the reduction of zinc oxide to metallic zinc is accomplished by the addition to the zinc oxide of some reducing agent as carbon, 10 a hydrocarbon or other organic compound which at elevated temperature combines with the oxygen of the zinc oxide to form zinc vapor and various proportions of water, carbon monoxide and carbon dioxide. These proportions are limited by 15 the respective chemical equilibria involved, and are determined by chemical reaction rates in approaching these equilibria. The zinc vapor is then condensed from this mixture by cooling. By this process as now practiced, it is not possible to obtain zinc entirely in a coherent form, 20 but some "blue powder" is always formed due to reversal at condensation temperatures of the above mentioned equilibria. This finely divided zinc and zinc-oxide mixture or blue powder is well known to owe its origin to mechanical as well as 25 chemical factors, (1) the rapid condensation of the zinc from the vapor to the solid or spheroidal state and (2) the reaction of the carbon dioxide, water or other oxygen compound formed by the 30 reduction reactions at higher temperatures with the zinc vapor or finely divided solid or spheroidal zinc metal particles when the temperature is lowered from the reduction temperature, to form zinc oxide which coats the zinc particles and 35 prevents coalescence. It will be seen from this discussion that if condensation takes place slowly the amount of powder due to factor one will be decreased but that formed by factor two will be increased so that the best that can be hoped for 40 is a compromise with the formation of considerable blue powder.

Other methods known to the prior art require the mixture of gases from the reduction of zinc oxide as above described to be passed over incandescent coke to remove the oxidizing gases before condensing the zinc. This method, however, requires the use of expensive solid fuel and requires two steps, the second of which must be carried out at a temperature considerably above 50 1000 degrees centigrade which offers difficulties of operation and produces less pure zinc than processes carried out at lower temperatures.

In still another method known in the prior art reducing gases such as carbon monoxide and 55 hydrogen are added to the condensing chamber. This involves an additional step in the preparation of the reducing gas and cannot substantially reduce the amount of oxidizing gas present without too much dilution of the zinc vapor which 60 causes difficulty in condensation. Carbon mon-

oxide and hydrogen in some instances have been used directly as reducing agents, but, such gases can reduce only insignificant amounts of zinc at temperatures below 1000° C. and the carbon dioxide or water vapor formed in the reaction 65 readily reoxidizes the metallic zinc when the mixed gases are cooled in the condenser to separate liquid zinc. In this process excessive amounts of blue powder invariably are obtained.

The principal object of my invention is the 70 provision of an improved process for producing metallic zinc.

Another object is to reduce zinc oxide by a 75 process in which no re-oxidizing vapor such as carbon dioxide or steam can be formed.

Another object is to reduce zinc oxide at lower 80 temperatures than have been used successfully heretofore.

Another object is to reduce zinc oxide to metallic zinc with the production of a minimum amount 85 of blue powder.

Another object is to reduce zinc by a process which can be carried out continuously and economically.

Other objects and features of the invention will 85 be apparent from the following detailed description taken with the accompanying drawings.

In the accompanying drawings I have illustrated in diagrammatic form two modifications of apparatus suitable for use in the practising of my 90 process. In this showing,

Figure 1 illustrates a suitable form of apparatus to be used when the pretreatment process hereinafter described is not employed in the practice of the invention, and

Figure 2 illustrates a modified form of apparatus for use when the pretreatment process hereinafter described is employed in conjunction with my process.

In general, my invention comprises the reduction of zinc oxide to metallic zinc by means of methane as a reducing agent, the source of the methane being preferably a natural gas which contains methane in amounts greater than approximately 80%. Other sources of methane 100 can, however, be employed.

In carrying out my process, I control all the factors so that the zinc oxide is reduced by the methane substantially according to the reaction



This reaction may be carried out in any suitable type of retort heated in any suitable manner to which the zinc oxide is supplied in relatively finely divided form. The gaseous products of the reaction are carried from the retort into a condenser where the zinc vapor is condensed and run off into suitable molds for further disposition in the usual way.

I am aware that the use of methane and other 120

hydrocarbons as reducing agents for zinc oxide has been suggested in the past, but by the methods heretofore disclosed it has not been possible to prevent the formation of a considerable percentage of carbon dioxide and water vapor due to side reactions such as



10

As previously disclosed, when such side reactions occur, it is impossible to prevent the formation of considerable amounts of blue powder, so much so in fact that the methane reduction of zinc oxide heretofore has been impracticable.

I have discovered, by the application of thermodynamic chemical methods to the equilibria involved in the reduction process, that by controlling certain factors including especially temperature and pressure, the disposition of the zinc oxide with respect to the methane and the absence of catalytic iron, in the condensing range, that I can substantially inhibit side reactions and the products of the reaction will be substantially zinc, carbon monoxide and hydrogen, with the formation of substantially no carbon dioxide or water vapor, with a concomitant decrease in the amount of blue powder formed. One of the most important characteristics of my invention is the discovery that methane will not decompose in the presence of zinc oxide, under the conditions herein described (but under other conditions methane is incapable of practical use for zinc reduction due to excessive decomposition into carbon and hydrogen). In other words, the rate of decomposition of methane in intimate contact with zinc oxide, within certain temperature ranges, is small as compared with the rate of reaction with zinc oxide. By making use of this discovery, and controlling the disposition of the methane with respect to the zinc oxide so that there is always an intimate contact between the two, the methane will be available in the form of  $\text{CH}_4$  for direct reaction with the zinc oxide. This, with a proper control of temperature, substantially completely avoids a possibility of side reactions of the character hereinabove referred to.

As to temperature, I have found that a temperature range of approximately 800° to 1000° centigrade produces the best results, with the very best temperature range between 925° to 990° centigrade. The following analysis will illustrate the results obtained in the preferred temperature range.

| Temperature (degrees centigrade) | Composition of outlet gas after condensing zinc— |      |                 |                |                  |
|----------------------------------|--------------------------------------------------|------|-----------------|----------------|------------------|
|                                  | CH <sub>4</sub>                                  | CO   | CO <sub>2</sub> | H <sub>2</sub> | H <sub>2</sub> O |
| 925                              | 23.3                                             | 25.0 | 0.5             | 51.2           | 0.7              |
| 940                              | 11.2                                             | 29.2 | 0.4             | 59.2           | 0.6              |
| 990                              | 0.0                                              | 32.5 | 0.8             | 66.7           | 0.9              |

Above this temperature range I have found that the carbon dioxide content increases and below it the methane decomposes with the deposition of carbon with consequent loss of efficiency.

By accomplishing the reduction within the above range and maintaining the methane throughout the heating range in intimate contact with the zinc oxide, I have secured excellent results in producing metallic zinc with

minimum amount of blue powder, substantially less than is customarily formed in the most satisfactory present commercial processes. The best results are obtained by a proper control of the condensing step of the process, particularly avoiding the presence of catalytic iron within the condensing range, and cooling at a controlled rate which is not too rapid, this being possible as hereinabove explained due to the fact that the gases entering the condenser consist substantially entirely of zinc, carbon monoxide and hydrogen. In actual practice, good results attend the practice of impinging the vapor stream directly upon the liquid zinc surface.

It is evident that the desirable reaction occurring between zinc oxide and methane is reversible but at the desirable temperatures set out the rate of the reducing reaction is so very much greater than the rate of speed of the reverse reaction that very high efficiency results and the yield of zinc vapor is relatively very large. It is, of course, true also that zinc oxide and carbon monoxide will react together in accordance with the following reaction



100

This reaction is undesirable as the presence of relatively large amounts of CO<sub>2</sub> in the condensing range will result in the formation of blue powder. This reaction also is reversible, however, and, at the temperatures which I select, chemical equilibria in this reaction are such as to prevent the formation of harmful amounts of carbon-dioxide. I have found that when the carbon dioxide content is kept below approximately 1% the rate of reoxidation reaction is so low that zinc vapor may readily be condensed without blue powder formation.

In this connection also the zinc oxide may, under certain conditions, react with hydrogen to form zinc vapor and water vapor. This water vapor is also undesirable in the condensation range because it also will cause the formation of blue powder. This reaction, however, is reversible according to the following reaction.



But, at the temperatures which I employ, only very slight traces of water vapor can be formed according to the equilibria involved, and slight traces of water vapor are without effect in the condensing range, as in the case of traces of carbon dioxide.

I shall now refer to the drawings in which I illustrate one type of apparatus with which my process may be carried out. I employ a retort 10 suitably supported within a furnace 11 into which retort the ore is adapted to be inserted through an ore delivery pipe 12. A gas delivery pipe 13 is provided adjacent the ore delivery pipe. The retort rests upon a condenser 14 and between the retort proper and the condenser I support in any suitable manner pieces of refractory material 16. Near the bottom of the retort proper 140 and above the pieces of refractory material I insert an ore discharge pipe 17 through which the residue of the ore, after the reduction of the zinc oxide, is passed. The gases, including the products of the reaction, pass through the refractory material 16 (which material holds back the ore) down into the condenser, its path through the condenser being relatively long due to the presence of horizontal baffles 18 and vertical baffles 19. The gases are cooled in their path through 150

the condenser and portions of the metallic zinc, becoming liquid, flow to the bottom of the condenser and out through a tap 21. The gases, however, impinge directly onto the liquid metallic zinc in the bottom of the condenser, and the uncondensed zinc vapor is changed to liquid coherent form.

The gases, including the carbon monoxide and hydrogen with the traces of other gases, pass out through a gas outlet 22. These outlet gases can be merely vented into the atmosphere, can be used to pre-treat the zinc ore, or can be used in other processes for example to remove sulphur from certain ores. It will be seen that with this form of apparatus the ore and gas may be fed continuously and concurrently or the retort may be charged with the ore and then reduced in a batch. I prefer, however, the continuous treatment for several reasons which readily suggest themselves, but principally because the "intimate contact" is more easily maintained with the continuous treatment.

One of the advantages of the concurrent downward movement of the ore and gas is that the intimate contact between the gas and ore is maintained. I have found that if this intimate contact is maintained, a metal retort can be used with satisfaction (the relatively low temperature also makes this possible) since whatever catalytic effect it may have is prevented by the anti-catalytic action of the zinc oxide on the methane. The use of a metal retort offers many advantages readily understood by those skilled in the art.

The intimate contact of gas with ore is an essential part of my invention. Thus, if a retort containing a zinc oxide ore containing cavities of appreciable size, or other unfilled spaces as, for example, a rotary kiln partly filled with ore charge, is subjected to the action of methane gas, I have found that the reduction is ineffective. Below 1000° C. substantially only carbon is formed by thermal decomposition of the hydrocarbon gas, and, at these temperatures, the carbon so formed will not subsequently react with zinc oxide to reduce the same. The carbon so formed would disappear at high temperatures by reaction with the zinc oxide in this way, but in doing so would produce reoxidizing carbon dioxide and the effect of my invention thus could not be obtained.

Methane gas is unstable at temperatures from 800-1000° C., but is effective for my purpose as controlled according to my teachings. I explain my results by the following hypothesis which seems to fit all of my findings. If attention is focused on an individual molecule of this gas, it is found that a certain critical time period after its temperature is raised (which in general is a major fraction of a second) is necessary to permit the reaction of decomposition to occur. If, however, this individual particle may be caused to come into contact with a molecule of zinc oxide before the critical time period has elapsed, the faster reaction of methane with zinc oxide takes place to the exclusion of thermal decomposition. I accomplish this conjunction of methane and zinc oxide in less than the critical time for thermal decomposition by maintaining it in intimate contact with the zinc oxide, preferably passing the gas downwardly through a finely granular bed of ore containing no large voids. Thus, if using briquetted charges, I partly fill the interstitial spaces with granular material passing through screens 8 meshes per inch, but remain-

ing upon screens 40 or 60 meshes per inch. In this way, the molecules of gas are never absent from ore particles for a great enough time to allow thermal decomposition.

The downward flow of gas makes the process relatively easily controllable since I have found that upward flowing gas tends to form channels in the ore charge, producing the voids which must be eliminated to prevent carbon formation.

The condenser is preferably made of a suitable refractory material substantially devoid of catalytic iron in its constitution. Many of the ordinary refractory materials of commerce are satisfactory for the purpose. The material indicated at 16 is, for example, broken pieces of refractory material. By saying that zinc oxide has an anti-catalytic effect, I mean that although methane is unstable at temperatures between 800° and 1000° centigrade, in the presence of zinc oxide and with sufficiently intimate contact, the reduction reaction may be made to occur preferentially as indicated above. For this reason, care should be taken to avoid raising the temperature of the methane to the reaction temperature in the absence of the anti-catalytic zinc oxide either before it enters the retort or even after entrance, and it should enter the retort at a point where the temperature is below 800 degrees for best results, although some slight preheating of the methane may take place without serious results. If care is not taken to maintain the methane in intimate contact with the zinc oxide, the carbon formed by the breaking down of the methane will be deposited in such a way as to substantially choke up the retort and prevent the proper movement of the gas therethrough. I found that once carbon starts to form it has a tendency to form relatively quickly but it will not initially begin to form if an ample supply of zinc oxide is present in substantially all portions of the retort in a condition to contact intimately with the methane.

Other ways of maintaining this intimate contact may, of course, be utilized in place of the down flow principle employed in the apparatus described. This is probably, however, one of the simplest means of obtaining the intimate contact and has been effective in producing very satisfactory results.

When I speak of the reduction of zinc oxide, it is understood that this term "zinc oxide" is employed in the usual manner customary in the industry. It includes roasted blend which has been substantially freed from sulphur or any natural or processed ore consisting essentially of zinc oxide.

One very satisfactory and novel way of practicing my invention is to employ the exit gases of the zinc oxide reduction process as they leave the retort for the pretreatment of the ore, as for example, for the removal of objectionable sulphur compounds and the like.

I have found that the small amounts of residual sulphur, which are usually from 0.5 to 2.0% in ores as customarily roasted for smelting, may cause serious difficulty in the methane reduction. A part of this sulphur, especially that part remaining as zinc sulphate in the roasted ore, is reduced by the gases to elementary sulphur gas, which mingles with the effluent gases of the retort and, coming in contact with liquid zinc in the condenser, recombines to form a fouled condensate containing infusible zinc sulphide. The material so formed is analogous to blue powder.

To avoid this trouble, I have found that I can remove the harmful sulphur impurities by pretreatment of the ore at temperatures slightly lower than 800° C., using the exit gases from the 5 retort, after condensation of the zinc therefrom. This pretreatment may be accomplished in another retort similar to the one used for reduction, but without the condenser, which is replaced by a settling chamber or dust separator to collect 10 the impurities driven off, and operated at temperatures approximately from about 600° to 800° C. Under these circumstances, practically no zinc is reduced. Some other substances may be affected by such pretreatment such as cadmium, 15 arsenic (if present), and some other volatile impurities.

I regard the pretreatment of ore by exit gases or other reducing gases of similar composition as an essential part of my process and as constituting 20 a part of the invention whereby blue powder formation is minimized, and entirely fusible and coherent substantially pure metallic zinc produced.

The ore is preferably fed to the retort at substantially 25 the temperature required to obtain the desired reaction described. In actually carrying out the process, the ore after roasting can be fed directly to the pre-treating retort and then to the reducing retort and this can be accomplished so that it will be at a temperature only slightly 30 below the reduction temperature when delivered to the reduction retort. If the pre-treatment step with the exit gas is not employed, any other suitable means may be employed for assuring that the ore is pre-heated before delivery to the reduction retort. The process can be carried on by supplying substantially cold ore to the reduction 35 retort and depend on the heat supplied to the retort to raise it to the reduction temperature, but this is not the preferred practice.

The reducing apparatus should be regulated to have a pressure slightly above atmospheric pressure to prevent the entrance of air at any point and it may be necessary under certain circumstances 45 to provide a small counter-current of the exit gas through the ore discharge pipe to prevent diffusion of zinc into such pipe.

In Figure 2 of the drawings, I have shown a modified form of apparatus for use when the pretreatment process described above is employed 50 in conjunction with my process. In this form of apparatus the construction is similar to that shown in Figure 1 with the exception that a pretreatment retort 30 is arranged above the retort 10 and is separated therefrom by a partition 31 in which a bell hopper 32 is arranged whereby pretreated ore may be delivered from the retort 30 to the retort 10 by operation of the lever 33. As will be apparent from Figure 2, in the modified form of apparatus shown the ore inlet pipe 12 is adapted to deliver ore into the retort 30 instead of directly into the retort 10, as in Figure 1. The gas outlet pipe 22, provided with a valve 34, is connected to the inlet side of a gas pump or fan 55 35 which is adapted to force the exit gases from the condenser through the pipe 36 to the gas inlet pipe 37 and into the pretreatment retort 30. Preferably at the lower end of the retort 30 and opposite the inlet pipe 37 is arranged a gas outlet pipe 38. As shown, the pipe 36 is also connected

with the pipe 39, having a valve 40, which connects with a gas inlet pipe 41 arranged in the ore discharge pipe 17, whereby a small counter-current of exit gas is provided in the ore discharge pipe 17 to prevent the diffusion of zinc into such pipe. 80

Those skilled in the art will understand that the explanation of the manner in which the process is carried out and in which the apparatus is constructed and operated is subject to considerable variation and modification in accordance with specific conditions. I do not restrict myself, therefore, in any sense by the details disclosed but the invention is limited only by the scope of the appended claims. 85 90

What I claim as new and desire to protect by United States Letters Patent is:

1. A process for reducing zinc oxide in ore to metallic zinc, which comprises continuously feeding zinc ore into the top of a vertically disposed retort, heating the ore to a temperature of between 800° C. and 1000° C., continuously supplying methane to the top of the retort and passing the methane vertically downwardly while maintaining intimate contact between the methane and zinc oxide in the heating range, whereby the methane and zinc oxide react to produce gaseous reaction products, including principally zinc vapor, carbon monoxide and hydrogen, passing the gaseous products into a condenser, condensing the zinc vapor and continuously removing residue ore material from the bottom of the retort. 100 105

2. A process for reducing zinc oxide to metallic zinc, which comprises continuously feeding the zinc oxide in relatively finely divided form into one end of a retort, heating the zinc oxide to a temperature between 800° C. and 1000° C., continuously passing methane into the same end of the retort as that into which the zinc oxide is delivered, whereby a concurrent and confluent movement of the zinc oxide and methane takes place through the retort, maintaining the zinc oxide and methane in intimate contact with each other in the heating range, whereby the methane is maintained stable with the exception of a reaction with zinc oxide to produce gaseous reaction products, including principally zinc vapor, carbon monoxide and hydrogen, passing the gaseous reaction products into a condenser to condense the zinc vapor and continuously removing solid residue material from the other end of the retort. 110 115 120 125

3. A process for reducing zinc oxide in ore to metallic zinc, which comprises continuously feeding zinc ore into the top of a vertically disposed retort, heating the ore continuously to a temperature between 800° C. and 1000° C., continuously supplying methane to the top of the retort and passing the methane vertically downwardly while maintaining intimate contact between the methane and zinc oxide in the heating range, whereby the methane and zinc oxide react to produce gaseous reaction products, including principally zinc vapor, carbon monoxide and hydrogen, passing the gaseous reduction products into a condenser substantially free of catalytic iron, condensing the zinc vapor, and continuously removing residue ore material from the bottom of the retort. 130 135 140

CHARLES G. MAIER. 145